

# United States Patent

Adwick et al.

[15] 3,688,242

[45] Aug. 29, 1972

[54] **SHUNT FOR OIL-IMMERSED CIRCUIT BREAKER**

[72] Inventors: **Albert Graham Adwick; Henry Nicholson**, both of North Shields, England

[73] Assignee: **Morganite Resistors Limited**, Jarrow, England

[22] Filed: **Oct. 21, 1970**

[21] Appl. No.: **82,683**

[30] **Foreign Application Priority Data**

Oct. 24, 1969 Great Britain.....52,145/69

[52] U.S. Cl. ....338/49, 200/146 R

[51] Int. Cl. ....H01c 13/00

[58] Field of Search.....338/20, 21, 49, 223-225; 317/9 R, 11 C, 11 E, 60; 200/144 R, 146 A, 146 R

[56]

References Cited

UNITED STATES PATENTS

|           |         |                      |           |
|-----------|---------|----------------------|-----------|
| 1,509,495 | 9/1924  | Slepian .....        | 338/21 X  |
| 2,305,577 | 12/1942 | Stoelting.....       | 338/21    |
| 2,281,385 | 4/1942  | Saint-Germain et al. | 200/146 R |

Primary Examiner—C. L. Albritton  
Attorney—Larson, Taylor & Hinds

[57]

ABSTRACT

The shunt of an oil-immersed circuit breaker is made of porous refractory conglomerate so that it becomes saturated with oil, whereby on passage of the high electric currents experienced with circuit breakers, the oil is rapidly heated and ejected from the pores to carry away energy at a high rate.

3 Claims, 4 Drawing Figures



Patented Aug. 29, 1972

3,688,242

2 Sheets-Sheet 1



FIG. 1

Patented Aug. 29, 1972

3,688,242

2 Sheets-Sheet 2



FIG. 2



FIG. 3



FIG. 4

## SHUNT FOR OIL-IMMersed CIRCUIT BREAKER

### DESCRIPTION

This invention relates to electrical resistance elements suitable for use in avoiding practical difficulties experienced with certain electrical equipment notably circuit breakers.

When an electric current is interrupted by a circuit breaker an arc may form between the separating contacts prolonging the current interrupting process. However, with high voltage apparatus, unless this arc occurs very high induced currents develop in inductive circuits associated with the circuit breaker. When circuit breakers are used in association with high voltage/high current apparatus, a very considerable quantity of energy is dissipated at each operation of the circuit breaker and its dissipation must be carefully controlled to avoid explosions or fires or damage to the apparatus. Two common methods of arc control are blowing out the arc with a blast of cold air and immersing the contacts in oil which has a high dielectric constant and can carry away heat energy.

Current control in circuit breakers can be assisted by connecting a resistor in shunt across the circuit breaker contacts and this invention provides an improved form of such shunt suitable for use with oil-immersed circuit breakers.

The improved shunt is formed so as to be permeable to a fluid so that on passage through the shunt of an electric current, the fluid with which the shunt is permeated is heated, and the shunt consists of a refractory conglomerate of at least two materials, respectively of a high and a low electrical resistivity, forming an open cellular structure having an apparent porosity not less than 25 percent and having a selected pore size.

In the use of such a fluid-permeable electrical resistance element as a shunt in an oil-immersed circuit breaker, the oil, which permeates and fills the pores, is rapidly heated by current passing through the element during circuit breaking and is expelled from the pores thereby rapidly carrying energy away from the element. Also, as is usual in oil-immersed circuit breakers, the oil, which has a high dielectric constant, helps to inhibit striking and restriking of an arc, for instance such as might occur between points formed by carbon particles on the surface of the resistance element.

The resistance element of this invention to be utilized as a shunt should have a total porosity of at least 25 percent and preferably between 25 and 30 percent, and the pores should be of a selected cross-sectional area such as to avoid disruptive failure on injection of such a large quantity of energy as would occur in circuit breaking. For instance, since the energy injection could be more than 2,000 joules/cc, the temperature of the element could be increased to about 1,000° C. in 100 milliseconds. Disruptive failure might occur due to high internal pressures developed due to such rapid heating of the oil if the pores are too small.

Also with most ceramics the pores should not be too large since this could lead to inferior performance either mechanically owing to the reduction in the number of bonds between granules, or electrically owing to surface tracking at lower voltages.

It is found that if the mean theoretical pore diameter is of the order of  $1.3 \pm 0.1$  microns for a porosity of the element of between 25 percent and 30 percent, exces-

sive pressure build-up in the pores is avoided. Such a pore size compares with a mean pore diameter of about 1.0 micron for a normal ceramic resistor.

The pores are merely required to be such as to enable the element to become oil saturated and to permit the oil to be expelled as above described when the circuit breaker operates. Thus the pores need not, but may, extend between two surfaces of the element.

A resistance element in accordance with the invention may be made largely by techniques known for making clay-carbon and similar electrical resistors except that care must be taken to avoid such vitrification of the material that its permeability is impaired.

In general, care should be taken to avoid the use of constituents, particularly binders, which vitrify on heating, a substantial proportion of relatively large particles of the basic refractory material should be included and only moderate pressures and a temporary binder, i.e. a volatile or combustible binder, should be used in forming the element to shape before firing.

In the manufacture of resistance elements of this invention, the pore size and permeability control can be effected by selecting the grain size of the mix of the conglomerate from which the shape is produced and carefully pressing the shape prior to firing.

Suitable clay-carbon conglomerates have the following general composition, by weight of starting materials, the proportions being varied to suit the electrical and fluid permeability requirements.

|                                                                                                                 |         |
|-----------------------------------------------------------------------------------------------------------------|---------|
| High Resistivity material                                                                                       |         |
| Particles of refractory material such as calcined clay, flints, zirconia, talc or alumina, or mixtures of these | 40-90%  |
| Low Resistivity material                                                                                        |         |
| Carbon                                                                                                          | 0.5-40% |
| Basic Binder                                                                                                    |         |
| Clay, such as ball clay, china clay or bentonite, or mixtures of these                                          | 3-50%.  |

The quantity of carbon used in the mix is selected to give the desired resistivity.

Methods of production of fluid-permeable electrical resistance elements of this invention will now be described in more detail.

The materials are thoroughly mixed, with or without water according to the kind of element to be made, formed to shape, such as by dry-pressing, moulding or extrusion and then fired, preferably between 1,200° and 1,400° C., in a non-oxidizing or reducing atmosphere. Mixing may be effected in any conventional ceramic mixer, e.g. a Planetary mixer or Sigma Blade mixer.

In the case of dry-pressing, a temporary binder, such as 3 percent w.w. ethylene glycol, may be used.

### EXAMPLE

The following describes by way of example one method of producing a shunt element.

A mix is produced comprising, in parts by weight:

|                                                                  |     |
|------------------------------------------------------------------|-----|
| Ceramic fillers (equal parts of calcined china clay and alumina) | 85  |
| Clay binder (equal parts of ball clay and bentonite)             | 15  |
| Carbon                                                           | 1.6 |

The ceramic fillers have a particle size up to about 10 microns diameter, the clay about 1 micron diameter and the carbon about 0.1 micron diameter. The ceramic ingredients are made up into a paste with water and the carbon added as a slip.

The mix is dried to between 6 and 7 percent moisture content as determined by a "Speedy Moisture Tester."

The mix so produced is next granulated by being forced through a sieve of selected mesh, e.g. 16, 18 or 22 B.S.S. mesh, and the resulting particles sieved on a smaller mesh sieve, e.g. 25, 30 or 36 B.S.S. mesh. The latter step may be omitted if the first sieving is carried out at such a speed that the particle size is about 0.50 mm and there is little distribution of particle size.

The sieve aperture sizes corresponding to the above B.S.S. mesh numbers are given in following table:

| Mesh No. | Aperture Size in mm |
|----------|---------------------|
| 16       | 1.00                |
| 18       | 0.85                |
| 22       | 0.71                |
| 25       | 0.60                |
| 30       | 0.50                |
| 36       | 0.425               |

The shapes to be fired are produced by pressing the granular material in punch dies to give a density of 2.35  $\pm$  0.05 gm/cm<sup>3</sup> corresponding to a fired density of about 2.2 gm/cm<sup>3</sup>.

The pressed shapes are then fired. Conveniently, for firing, the shapes are packed in saggars containing loose carbon material, e.g. graphite or broken coke, which combines with any oxygen in the furnace to provide an inert atmosphere. The temperature of firing is between 1,200° and 1,400° C., the temperature employed determining the degree of sintering.

Finally, the surfaces are metallized as required. Also the fired shape may have its peripheral surface treated with an anti-tracking coating.

In tests, using a resistance element having a resistivity of 250 $\Omega$  inch pressed from particles pressed through an 18 B.S.S. mesh sieve and retained on a 30 B.S.S. mesh sieve and pressed to a density of 2.37 gm/cm<sup>3</sup>, the following results were obtained:

| Time of voltage duration at 50Hz (milliseconds) | Applied voltage at disc failure kV(rms) per inch |
|-------------------------------------------------|--------------------------------------------------|
| 45                                              | 8.1                                              |
| 85                                              | 7.1                                              |
| 115                                             | 6.1                                              |
| 175                                             | 5.1                                              |
| 245                                             | 4.6                                              |

The stability after energy injection was as follows:

| Energy injection (joules/cc) | Injection Time (ms) | % Resistance Change |
|------------------------------|---------------------|---------------------|
| 390                          | 200                 | +0.19               |
| 500                          | 300                 | +0.22               |
| 530                          | 300                 | +0.22               |
| 560                          | 350                 | +0.16               |

The elements, which are conveniently cylindrical, may be 3 inches in outside diameter, and 1 inch long with a 1-inch diameter bore and in use a number of these may be threaded on to an insulating rod to give a resistor value of 15 ohms for circuit breakers in 5 to 6 kV supplies.

This invention therefore comprises the production of fluid permeable electrical resistance elements having a mean theoretical pore diameter of the order of 1.3 microns for a porosity of 25 to 30 percent, and comprises also the combination of such elements with oil-filled circuit breakers in shunt across the circuit breaker contacts.

The accompanying drawings illustrate by way of example an oil-filled circuit breaker and one form of shunt of this invention.

In the drawings,

FIG. 1 is a diagrammatic section through the circuit breaker,

FIGS. 2 and 3 shown in plan and elevation a typical shunt element, and

FIG. 4 shows a shunt such as may be used in a circuit breaker as shown in FIG. 1.

Referring to FIG. 1, a typical oil-filled circuit breaker comprises an oil-containing tank 10 having mounted on it insulating bushes 11 for conductors 14 by which the circuit breaker is connected in the power line to be protected. From the inner ends of the bushes 11, the conductors 14 lead to a pair of fixed contacts 12 of the circuit breaker, these contacts being in separate explosion pots 13. When the circuit breaker is closed, the contacts 12 are connected electrically by a bridging conductor 15 having at its ends rod-like moving contacts 16 which project into the explosion pots 13 into contact with the fixed contacts 12.

The bridging conductor 15 is carried by an operating mechanism including a downwardly-movable, insulating operating-rod 17. In operation, on downward movement of the rod 17, the contacts 16 separate from the contacts 12 and are withdrawn from the pots 13 and during this movement arcs form between the contacts, the energy of the arcs being dissipated by heating and vaporizing the oil in the explosion pots 13. The vapors and gases generated assist to prevent the arc from reforming.

According to this invention, there are also provided electrically-conductive shunts 20 formed from elements as described above.

One such element 21 is shown in FIGS. 2 and 3, and it consists of a porous ceramic ring of say 6 inches diameter and 1 inch thickness and having a bore of 1.4 inches diameter, the outer and inner edges 22, 23 being chamfered and the flat surfaces being metallized but with a gap left between the edges of the metallization 24 and the chamfers.

A shunt may conveniently comprise a 10-inch stack 25 of such elements 21 mounted on an insulating rod 26.

We claim:

1. A shunt for use in an oil-immersed circuit breaker which shunt is permeable to the oil so that in use on passage of an electric current through the shunt the oil is heated, the shunt comprising a refractory conglomerate of particles of at least two materials, respectively of relatively a high electrical resistivity and a low

electrical resistivity, forming an oil-permeable open cellular structure having an apparent porosity of the element between 25 and 30 percent, the pores having a mean pore diameter of  $1.3 \pm 0.1$  microns giving a cross-sectional area such as to avoid disruptive failure on injection of such a large quantity of energy as would occur in circuit breaking.

2. An oil-immersed circuit breaker having separable electrical contacts and a shunt connected across the contacts and carrying current during separation of the contacts, the shunt comprising a refractory conglomerate of particles of at least two materials, respectively of relatively a high electrical resistivity and a low electrical resistivity, forming an oil-permeable open cellular structure having an apparent porosity of the element between 25 and 30 percent, the pores having a mean pore diameter of  $1.3 \pm 0.1$  microns giving a cross-sectional area such as to avoid disruptive failure on injection of such a large quantity of energy as would occur in circuit breaking.

3. A shunt for use in an oil-immersed circuit breaker which shunt is permeable to the oil so that in use on

passage of an electric current through the shunt the oil is heated, the shunt comprising a refractory clay-carbon conglomerate of particles, the conglomerate having the general composition, by weight of the starting materials:

|                                                                   |         |
|-------------------------------------------------------------------|---------|
| High Resistivity Material                                         |         |
| Particles of refractory material such as calcined clay or alumina | 40-90%  |
| Low Resistivity Material                                          |         |
| Carbon                                                            | 0.5-40% |
| Basic Binder                                                      |         |
| Clay, such as ball clay and/or bentenite                          | 3-50%,  |

15 said clay being of relatively a high electrical resistivity and said carbon having a low electrical resistivity, forming an oil-permeable open cellular structure having an apparent porosity of the element not less than 25 percent the pores being of a selected cross-sectional area such as to avoid disruptive failure on injection of such a large quantity of energy as would occur in circuit breaking.

\* \* \* \* \*

25

30

35

40

45

50

55

60

65